

1

2,822,259

## METHOD OF PRODUCING REFRactory METALS

Bertram C. Raynes, Euclid, Ohio, assignor, by mesne assignments, to Horizons Titanium Corporation, Princeton, N. J., a corporation of New Jersey

No Drawing. Application August 13, 1954  
Serial No. 449,802

7 Claims. (Cl. 75—84.1)

This invention relates to the production of certain refractory transition metals and, more particularly, to the production of these metals by pyrolytic reduction of a complex fluoride of the metal with carbon or the carbide of the metal.

All attempts heretofore to produce metallic titanium by reduction of any of its compounds with carbon appear to have met with failure because of the pronounced tendency for metallic titanium to combine with carbon to form titanium carbide. Consequently, the recent attempts to produce metallic titanium have been directed either along the lines of electrolytic reduction or the reduction of a halide of the titanium with a metal such as magnesium, calcium, sodium, or the like. In all of these procedures, the metallic titanium which is produced is obtained in the form of fine particles enshrouded in a mass of various salts, and the problems associated with the recovery of this metallic titanium in a massive form have proven to be nearly as formidable as the problem of producing the metal from titanium compounds. While titanium has been mentioned herein by way of example, it is well known that many of the other transition metals are similarly refractory.

I have now discovered that certain refractory transition metals may be obtained in the metallic state by the reduction of their alkali metal double fluorides with carbon or with the carbides of these transition metals at elevated temperatures. And contrary to expectations, I have found that the metal so produced is substantially free of carbon either in the free state or as the metal carbide. I have found that this method is applicable to the production of the transition metals of the group consisting of titanium, zirconium, hafnium, vanadium, niobium, tantalum, uranium, molybdenum, tungsten and chromium. The method of my present invention comprises effecting contact between either carbon or the carbide of one of these transition metals and a molten body consisting essentially of an alkali metal double fluoride of one of the transition metals at a temperature of about 1800° C. and higher. This contact promotes reduction of the double fluoride with the resulting formation of the transition metal in the molten body of reactant salts. However, because of the high temperature employed in the practice of my invention, which is above the melting points of many of the aforementioned metals, it is possible by the practice of my invention to form and collect such metals in the molten state so as to be recoverable from the reactant salt mass in a massive form.

The alkali metal double fluorides of the aforementioned transition metals may be either the sodium, potassium or lithium double fluorides. These double fluorides are stable at the elevated temperatures required in the practice of my invention and are furthermore readily obtainable. Although these double fluorides may be used in their commercially available form for the practice of my invention, I have found it advisable to use these fluorides in as pure a form as is convenient. All of these

2

double fluorides can be readily purified by conventional recrystallization techniques and even the single-recrystallized products are remarkably pure. If desired, for control of the fluidity or volatility of the double fluoride melt, or simply as a carrier for the double fluoride, an alkali metal halide may be admixed with the double fluoride.

The carbonaceous material which is used to reduce the aforementioned double fluorides in practicing my invention consists either of carbon or of the carbide of the transition metal. The carbon may be added to the double fluoride either in the form of finely divided carbon or, where the heat for the reaction is to be provided by an electric arc, the carbon electrode may serve as the source of carbon. When a transition metal carbide is used as the carbonaceous reducing material, I have found it generally advisable to add this carbide to the double fluoride in finely divided form although the carbides can be formed into electrodes and be used in the same way as carbon electrodes. Most of the transition metal carbides melt at temperatures above 1800° C. and thus effectively present their carbon component for reaction with the double fluoride.

The reaction between the transition metal double fluoride and the carbonaceous reducing material can be illustrated by the following reaction which is directed specifically to the reduction of potassium titanium fluoride with carbon:



As can be seen from this equation, the products of the reaction comprise the transition metal itself, potassium fluoride and carbon tetrafluoride. Inasmuch as the metal separates from the fused salt and inasmuch as the carbon tetrafluoride is promptly evolved from the molten reaction mass, these products are formed to the extent permitted by the amount of either of the two reactants. Accordingly, it is not necessary that the reactants be introduced into the reaction zone in stoichiometric amounts provided that an excess of free carbon does not remain in the final reaction product. That is, it is generally advisable to use an excess of the alkali metal double fluoride of the transition metal in order to assure complete utilization of all carbonaceous reducing material available in the reaction zone. As long as there is a significant amount of the alkali metal-transition metal double fluoride available for reaction with the carbon, there appears to be no observable tendency for the carbon to combine preferentially with the transition metal which has been formed as a result of the reaction. Therefore, the transition metal which is produced by the practice of my invention is virtually uncontaminated by carbon. If, however, the reaction is carried out under conditions which present an excess of carbon over the amount required to reduce the alkali metal-transition metal double fluoride, the carbon or carbide present in the resulting transition metal product can be removed by using this carbon-contaminated metal either as a source of the carbonaceous material for reaction with another mass of the double fluoride or it can be used as the solid transition metal anode which is electrolyzed pursuant to the invention described and claimed in the copending application of Merle E. Sibert et al., Serial No. 358,194, filed May 28, 1953.

The reaction between the double fluoride and the carbonaceous reducing material requires reaction temperatures of about 1800° C. and higher, and in general I have found that temperatures within the range of about 1800° to 2500° C. are effective. These relatively high reaction temperatures may be obtained by any means capable of supplying the necessary amount of heat. For example, the reaction heat may be provided by an arc struck between two carbon or transition metal carbide electrodes

immersed in a mass of the alkali metal-transition metal double fluoride. The arc not only fuses the double fluoride and brings it up to reaction temperature in the neighborhood of the arc, but the electrodes further supply the carbonaceous material for the reduction reaction. On the other hand, the heat for reaction may be provided by external heating elements or by using the bath itself as a resistance element by passing current through the bath.

The reaction vessel in which the alkali metal-transition metal double fluoride is reduced by the carbonaceous material pursuant to my invention may be constructed of any material that is non-reactive with respect to the reactants at the temperature at which contact is effected between the reactants and the vessel. The problem of selecting such a material is completely eliminated, however, by using a water-cooled metal shell as the reaction vessel so that the interior of the shell is protected by a wall or skull of the double fluoride salt in the solid state. By means of such an expedient, there is complete assurance that the product metal will not be contaminated by extraneous impurities.

The transition metal product obtained by the practice of my invention may be in either the finely divided or massive form. If, as in the case of titanium, zirconium, vanadium, uranium and chromium (all of which have melting points not in excess of about 1900° C.), the reaction temperature exceeds the melting point of the transition metal, the metal will be formed in the molten state and will liquefy into a mass of the metal and thus be recovered in the form of a pig. On the other hand, a less massive form of the transition metal will be obtained when the metal has a melting point higher than the reaction temperature. In either case, it may be desired to obtain the transition metal in alloyage with one or more other metals, and in this event, by incorporating such other metal or metals in the reaction mass there will be obtained an alloy of the transition metal which will usually have a lower melting point than that of the transition metal. Of course, the alloying metal need not be other than another transition metal, and if such an alloyage of two or more transition metals is desired it can be obtained by the practice of this invention by using a mixture of the corresponding transition metal double fluorides or by using the carbides and double fluorides of different transition metals as the reactants, or by a combination of these techniques.

In addition to the production of the aforesaid transition metals, the method of my invention produces an equivalent amount of carbon tetrafluoride. Inasmuch as the carbon tetrafluoride does not decompose and liberate fluorine which might otherwise react with the produced transition metal, this tetrafluoride serves as a protective atmosphere for the metal as it is formed. Still further protection of the metal may be obtained by admitting to the reaction vessel a gas such as pure, dry argon or helium which is inert with respect to the reactants and the reaction products at the prevailing reaction conditions, or a reducing atmosphere containing hydrogen may be used. Still further protection of the reaction zone may be obtained by maintaining on the surface of the molten double fluoride a fresh charge of this double fluoride in granular form. Such a protective blanket of solid-state salt further serves to collect and retain any volatilized salt formed in the reaction zone.

The carbon tetrafluoride produced in practicing my invention can, I have further found, be used to convert the transition metal component of such a metal carbide to the transition metal tetrafluoride (or corresponding high valence fluoride). This conversion takes place generally at temperatures of about 900° to 1200° C., particularly when a small amount (generally about 2% by weight) of elemental chlorine is present. The products of such a conversion reaction are solid carbon and vapors of the transition metal fluoride, and therefore the transition metal fluoride vapors may be readily formed simply

by passing the carbon tetrafluoride vapors through or over a body of the transition metal carbide in finely divided form under the aforementioned conditions. The transition metal tetrafluoride may also be produced by reacting the carbon tetrafluoride with an oxide (such as the monoxide, sesquioxide or dioxide) of the transition metal at a temperature within the range of about 1000° to 1400° C. If it is desired to use the resulting transition metal tetrafluoride for the regeneration of the corresponding alkali metal-transition metal double fluoride, the tetrafluoride may be dissolved in dilute aqueous hydrofluoric acid, and potassium fluoride is then added to the resulting mixture to form the potassium-transition metal double fluoride which can be recovered by crystallization or salting out from the reaction medium.

The carbon tetrafluoride may be used in other ways to regenerate the alkali metal-transition metal double fluoride. For example, the tetrafluoride may be passed into molten potassium hydroxide (with evolution of carbon dioxide), and the resulting potassium fluoride is then added to a mixture or solution of the transition metal dioxide (or other transition metal compound) in dilute aqueous hydrofluoric acid. The hydrofluoric acid may be obtained from an extraneous source or it may be produced by reaction between the carbon tetrafluoride and either water or hydrogen.

If the transition metal product obtained by the practice of my invention is for any reason contaminated by an excess of the transition metal carbide, the contaminated metal may be brought in finely divided form into contact with a molten mass of the same transition metal-alkali metal double fluoride as described in the copending application of John T. Burwell, Jr., and Quentin H. McKenna, Serial No. 398,193, filed December 14, 1953, whereupon the transition metal component of the carbide will be transformed to one or more lower valent transition metal fluorides. These fluorides are then removed from the residual carbide-free transition metal product by leaching, volatilization, or the like.

Thus, it will be appreciated that the method of my invention is particularly adapted to produce the aforementioned transition metals in substantially pure condition and, in the case of some of these metals such as titanium, in a massive state. It will also be appreciated that the transition metal carbide which is reacted with the double fluoride in accordance with the invention may be the carbide which contaminates an otherwise substantially pure transition metal, and therefore the method of my invention can be used to effect purification of carbide-containing transition metals.

The following examples are illustrative, but not limitative, of the practice of my invention:

#### Example I

Sodium chloride was melted by resistive heating in a graphite crucible. When the sodium chloride was molten, potassium titanium fluoride ( $K_2TiF_6$ ) was added in solid form to this bath. The A. C. voltage on the graphite electrodes, which performed the double function of electrode and carbon source for the reaction, was then increased to about 40 volts so that an arc was formed under the molten bath surface. Additions of the double fluoride were continually made and as the graphite electrodes were consumed they were lowered further into the fused bath. Upon completion of the reaction, the molten mixture was allowed to solidify and cool to room temperature. The solid mixture was leached by simple aqueous techniques and a finely divided, thermally produced titanium powder was recovered having a purity of about 98%. X-ray analysis of the metal powder revealed the presence of no titanium carbide.

#### Example II

A mixture of potassium titanium fluoride and carbon black was placed in a graphite crucible and a direct current arc was struck and maintained between graphite

electrodes over this crucible and out of contact with the charge. Upon subsequently cooling the fused crucible charge, the mass in the crucible was removed and leached. Titanium powder of similar high purity was thus recovered.

I claim:

1. The method of producing a substantially carbon-free metal of the group consisting of titanium, zirconium, hafnium, vanadium, niobium, tantalum, uranium, molybdenum, tungsten and chromium which comprises effecting contact between (a) a carbonaceous material of the group consisting of carbon, carbon-contaminated transition metal and carbides of said metals and (b) a molten body consisting essentially of an alkali metal double fluoride of said metal at a temperature of about 1800° C. and higher, and recovering the resulting metal formed in said molten body.

2. The method of producing a substantially carbon-free metal of the group consisting of titanium, zirconium, hafnium, vanadium, niobium, tantalum, uranium, molybdenum, tungsten and chromium which comprises effecting contact between (a) a carbonaceous material of the group consisting of carbon, carbon-contaminated transition metal and carbides of said metals and (b) a molten body consisting essentially of an alkali metal double fluoride of said metal at a temperature of about 1800° to about 2500° C., and recovering the resulting metal formed in said molten body.

3. The method of producing a substantially carbon-free metal of the group consisting of titanium, zirconium, hafnium, vanadium, niobium, tantalum, uranium, molybdenum, tungsten and chromium which comprises effecting contact between (a) a carbonaceous material of the group consisting of carbon, carbon-contaminated transition metal and carbides of said metals and (b) a molten body consisting essentially of an alkali metal double fluoride of said metal at a temperature of about 1800° C. and higher obtained by an arc struck between electrodes of said carbonaceous material below the surface of said molten body, and recovering the resulting metal formed in said molten body.

4. The method of producing carbon tetrafluoride which comprises effecting contact between (a) a carbonaceous material of the group consisting of carbon and carbides of a transition metal of the group consisting of titanium, zirconium, hafnium, vanadium, niobium, tantalum, uranium, molybdenum, tungsten and chromium and (b) a molten body consisting essentially of an alkali metal double fluoride of said metal at a temperature of at least about 1800° C., and recovering the resulting vapors of carbon tetrafluoride evolved from said molten body.

5. The method of purifying a transition metal of the

group consisting of titanium, zirconium, hafnium, vanadium, niobium, tantalum, uranium, molybdenum, tungsten and chromium to effect the removal of contaminating carbon therefrom which comprises effecting contact between

5 said carbon-contaminated transition metal in finely divided form and a molten body consisting essentially of an alkali metal double fluoride of said metal at a temperature of about 1800° C. and higher, and recovering the resulting carbon-free transition metal from the molten salt mass.

6. The method of producing an alloy of a substantially carbon-free metal of the group consisting of titanium, zirconium, hafnium, vanadium, niobium, tantalum, uranium, molybdenum, tungsten and chromium which

15 comprises effecting contact between (a) a carbonaceous material of the group consisting of carbon and carbides of said metals, (b) a molten body consisting essentially of an alkali metal double fluoride of said metal, and (c) a metal with which the transition metal is to be alloyed, 20 at a temperature of about 1800° C. and higher, and recovering the resulting alloy metal formed in said molten body.

7. The method of producing substantially carbon-free metal of the group consisting of titanium, zirconium, 25 hafnium, vanadium, niobium, tantalum, uranium, molybdenum, tungsten and chromium from a carbide of said metal which comprises bringing the carbide of said transition metal into contact with carbon tetrafluoride and elemental chlorine at a temperature within the range

30 of about 800° to 1800° C., bringing the resulting transition metal fluoride into admixture with an alkali metal fluoride in the presence of aqueous dilute hydrofluoric acid with the resulting formation of the corresponding alkali metal-transition metal double fluoride, recovering

35 the double fluoride from the resulting aqueous reaction mass, effecting contact between the recovered double fluoride in the form of a molten body thereof and a carbonaceous material of the group consisting of carbon, carbon-contaminated transition metal and carbides of

40 the transition metals at a temperature of about 1800° C. and higher, recovering the resulting evolved carbon tetrafluoride, and recovering the resulting transition metal formed in said molten body.

45 References Cited in the file of this patent

UNITED STATES PATENTS

|           |                |               |
|-----------|----------------|---------------|
| 2,639,218 | Anderson       | May 19, 1953  |
| 2,692,186 | Kamlet         | Oct. 19, 1954 |
| 2,694,616 | Wainer         | Nov. 16, 1954 |
| 2,694,617 | Cardon et al.  | Nov. 16, 1954 |
| 2,703,752 | Glasser et al. | Mar. 8, 1955  |
| 2,708,158 | Smith          | May 10, 1955  |